

## UNITED STATES PATENT OFFICE

2,014,235

## TREATMENT OF MOTOR FUEL

Charles D. Lowry, Jr., Chicago, Ill., assignor to  
Universal Oil Products Company, Chicago, Ill.,  
a corporation of Delaware

No Drawing. Application February 5, 1934,  
Serial No. 709,791

7 Claims. (Cl. 44—9)

This invention relates more particularly to the treatment of motor fuel either consisting entirely of or containing substantial percentages of the lighter distillates produced in cracking operations upon the heavier distillate and residual portion of petroleum oils though the treatment may also be utilized in connection with motor fuels produced from other raw hydrocarbon sources such as shale oil, coal, etc.

More specifically the invention is concerned with a particular method of treatment which insures the preservation of the more desirable properties of motor fuel while under storage conditions. This is accomplished by the use of novel materials whose value in this connection has been hitherto unsuspected.

Until cracked motor fuels were produced in appreciable quantities to augment the failing supply of straight run gasolines, no special difficulties were encountered in the loss of desirable characteristics on storage as evidenced by the development of undesirable color and high gum content and loss in anti-knock value since the straight run gasolines, even if produced by poorly controlled distillation methods, contained little or no amount of sufficiently unsaturated hydrocarbons which were susceptible to oxidation under storage conditions. Cracked gasolines, however, have been shown to contain sufficient percentages of diolefins and similar compounds to account for at least the major portion of the observed depreciation of gasolines under storage conditions, these compounds forming peroxides initially by direct addition of oxygen to conjugated double bonds. These peroxides then instigate a series of chain reactions which result in the formation of colored bodies, gums and resins and evidently account for the observed deterioration in anti-knock properties.

Chemical treatments aimed at the removal of the unstable hydrocarbons frequently entail the loss of large percentages of distillates and are costly and cumbersome, so that recently a great deal of work has been done in the industry with the object of developing numerous types of soluble antioxidant materials which eliminate the necessity for chemical treatment and inhibit the effect of oxygen upon the gasolines by exerting for a time at least a preferential affinity therefor. The present invention is a contribution to the inhibitor art involving the use of material which is readily available, inexpensive and effective not only as an inhibitor but also in other ways as will be disclosed in succeeding paragraphs.

In one specific embodiment the invention com-

prises the use of unrefined corn oil as an inhibitor in unstable gasolines, particularly cracked gasolines.

I have determined by experiments, the results of which will be given later that crude corn oil produced by extraction or pressing of the corn germ contains considerable percentages of compounds which have an antioxidant action. This is evidenced primarily by the fact that unrefined corn oil itself possesses greater stability against rancidity than the refined product which has usually been treated with alkalies to remove acidic and other types of organic compounds. Compounds which are evidently responsible for the observed antioxidant action are apparently the sterols which frequently comprise from 2 to 3% of the crude oil. The chemical character of these compounds merits some special attention.

The sterols have a complicated chemical structure and are usually considered as cyclic alcohols of high molecular weight. They differ chemically from the aliphatic alcohols most essentially in that they are not converted into fatty acids having the same number of carbon atoms by heating with soda, lime and similar alkaline reagents. Some of the representative members of this class of compounds are shown below:

Cholesterol, phytosterol (sitosterol), stigmasterol, brassicasterol, coprosterol.

Of the members of the above group cholesterol has been studied most extensively and is generally considered to be a complicated terpene compound having the formula  $C_{27}H_{46}O$ . Structurally it is represented as follows:

(Lewkowitsch)



The other members of the group have the same general formula but differ slightly in their structural arrangement. It is most likely that the particular sterol in corn oil is sitosterol, the presence of which has also been detected in oils from wheat and other grains. Cholesterol has thus far not been detected in vegetable oils, in fact, its presence is commonly considered as prima facie evidence of the animal origin of an oil or fat.

In utilizing the process of the invention to treat and stabilize cracked gasolines, amounts of corn oil varying from 1 to approximately 5% are dissolved in the gasoline. The major portion of the oil which consists of fatty acid esters performs a further useful function in that it assists in lubricating the top portion of the cylinders of the internal combustion engine in which the fuel is

- burned. The exact amount of any corn oil necessary for stabilizing a given gasoline will depend upon the chemical composition of the gasoline and its resistance to oxidizing influences. Furthermore, the actual inhibiting value of corn oils from different sources will vary so that different amounts will be required to effect an equivalent stabilization of properties in the same gasoline. The necessary amounts may be readily determined by small scale laboratory tests involving the determination of the induction period in the oxygen bomb test and the change in gum content and antiknock value of the gasoline before and after the test.
- 15 As an example of results obtainable by using corn oil as an inhibitor in gasoline the following is cited though other examples are numerous and the invention is not limited by the particular data given.
- 20 A paraffinic cracked gasoline was found to have an induction period of only 45 minutes in the oxygen bomb. The addition of 0.5% by volume of corn oil raised the induction period to 180 minutes and the addition of 2.5% of corn oil raised the induction period to 400 minutes, the latter figure being considerably in excess of the 240 minute requirement which is generally conceded to indicate a practical 6 months' storage stability.
- 25 The scope of the invention and the character of the results obtained by its use are evident from the foregoing specification and single numerical example and it is to be understood that neither is to be construed in the light of imposing undue limitations thereon.
- 30 I claim as my invention:
- 35 1. A process for the treatment of hydrocarbon oil containing readily oxidizable unsaturates to

prevent deterioration thereof in respect to gum and color formation, which comprises adding to the said hydrocarbon oil a small quantity of an unrefined corn oil.

2. A process for the treatment of cracked hydrocarbon oil to prevent deterioration thereof in respect to gum and color formation and deterioration of anti-knock properties, which comprises adding to the said cracked hydrocarbon oil a small quantity of an unrefined corn oil. 5

3. A process for the treatment of hydrocarbon oil containing readily oxidizable unsaturates of substantially gasoline boiling range to prevent deterioration thereof in respect to gum and color formation and deterioration of anti-knock properties, which comprises adding to the said hydrocarbon oil a small quantity of an unrefined corn oil. 10

4. A process for the treatment of cracked gasoline to prevent deterioration thereof in respect to gum and color formation and deterioration of anti-knock properties, which comprises adding to the said cracked gasoline a small quantity of an unrefined corn oil. 20

5. A method for preventing deterioration of hydrocarbon material containing readily oxidizable unsaturates, which comprises adding to the hydrocarbon material a small quantity of unrefined corn oil. 25

6. A method for stabilizing motor fuel containing unsaturated hydrocarbons produced by cracking, which comprises adding to the motor fuel a small amount of unrefined corn oil. 30

7. Motor fuel comprising cracked gasoline containing a relatively small amount of unrefined corn oil. 35

CHARLES D. LOWRY JR.